# EUROPEAN PATENT SPECIFICATION

(11) **EP 1 392 923 B1**
(45) Date of publication and mention of the grant of the patent: **25.07.2018**
(21) Application number: 02718226.0
(22) Date of filing: 24.04.2002
(51) Int. Cl.: D21H 17/69, D21H 27/38

(54) **MULTILAYERED FIBROUS PRODUCT AND A PROCESS FOR THE PRODUCTION THEREOF**
MEHRSCHICHTIGES FASERPRODUKT UND VERFAHREN ZU SEINER HERSTELLUNG
PRODUIT FIBREUX MULTICOUCHE ET SON PROCEDE DE PRODUCTION

(30) Priority: 24.04.2001 FI 20010848
(43) Date of publication of application: 03.03.2004
(73) Proprietor: Metsä Board Oyj, 02100 Espoo (FI)
(72) Inventor: SILENIUS, Petri, FIN-08500 Lohja as. (FI); YLINIEMI, Leena, FIN-94100 Kemi (FI); MEURONEN, Jari, Par, Cornwall PL24 2 PQ (GB); LESKELÄ, Markku, FIN-08500 Lohja as. (FI)
(74) Representative: Seppo Laine Oy
(86) International application number: PCT/FI2002/000342
(87) International publication number: WO 2002/092910

(56) References cited:
- EP-A2- 0 791 685
- EP-A2- 0 930 345
- WO-A1-96/36750
- WO-A1-97/01670
- GB-A- 628 603
- US-A- 5 223 090
- US-A- 5 824 364

## Description

The present invention concerns a multi-layer fibrous product according to the preamble of claim 1.

This kind of a product comprises at least two overlapping fibrous layers, of which at least the layer forming the operating surface of the product is light and essentially opaque (non-transparent), covering the fibre layer under it. The top layer contains filler and possibly conventional additives and auxiliary agents for paper.

The present invention relates also to a process according to claim 8 for producing of multi-layer fibrous product.

A multilayered fibrous product usually consisting of two or three layer is called a "liner". A liner can be completely brown (kraft-liner) or partially white (white-lined liner) or its top layer can be coated. The liner can be made of virgin fibre or recycled fibre or both.

A liner is used as a surface of a background liner in a corrugate board package. The special characteristics of kraft-liners are strength, uniform quality and product safety. Strength is with kraft-liners a very important competitive advantage when comparing with recycled fibre-based products. The advantages of using test liners that contain recycled fibre are low price and the ecological values that support recycling.

The products called "Kemiart Graph" and "Kemiart Lite" and the uncoated "Kemiart Brite" of Oy Metsä-Botnia Ab can be mentioned as examples of commercial coated liners. The liner product of Oy Metsä-Botnia Ab is a kraft-liner that has two fibre layers, the base layer being high yield softwood sulphate pulp and the top layer of bleached birch and softwood sulphate pulp. The fillers are used in the top layer to give the surface more brightness and smoothness, which improves the printability properties. Other chemicals, such as retention agents, are also used in production of liner, in order to retain the noil material and filling agents in the product instead of cycling it in the water cycle, and AKD adhesives to improve water resistance. The coating is added to the coated products with an on-line coating unit. The coating is, for example, a combination of kaolin, carbonate and latex which improves significantly the printability of the product. The final gloss and smoothness of the final product are obtained with calendering.

The method of producing the top layer of the white lined linerboard (cover layer) is considerably more expensive than the method of producing brown back layer. The product can be optimised by changing, for example, the strengths of the fibre layers. In that case it would be reasonable to produce the liner the top layer of which is as lightweight as possible. So far, however, the attempts to reduce the weight of the cover while maintaining a sufficient brightness of a liner without making the cover too weak, have been unsuccessful. The amount of the white fibre cannot be decreased easily, without the brown fibre showing through.

The top layer does also need to have a good formation, which shows directly as good printability. Thus bad formation is visible especially well in grey scales of offset printing and as mottled print quality.

It is an object of the present invention to eliminate the problems involved with the known methods and to provide a novel solution for producing multi-layer fibre products, such as liners.

The present invention is based on the idea that a composite filler consisting of fibrils and mineral pigments is used as a filler of the top layer of the fibre product mentioned in the introduction.

Finnish Patent Specification No. 100729 discloses a papermaking filler comprising porous aggregates formed by precipitated calcium carbonate particles on the surface of fines. What characterises this new kind of filler is that, according to the patent specification, the calcium carbonate is precipitated on fine fibrils produced by refining cellulose fibres and/or mechanical pulp fibres. The size distribution of the fines fraction corresponds mainly to the wire screen fraction P100.

According to the present invention, it has been found that when the top layer of a multi-layer product is filled with the filler described above, the opacity of the surface increases so drastically that the grammage of the cover can be reduced significantly. The top layer containing the new filler covers very efficiently the brown background despite the lower grammage.

Furthermore, within the scope of the present invention it has been found that also other similar fillers consisting at least partly of cellulose or lignocellulose fibrils, over which light scattering material particles has been precipitated, can be used as fillers. These particles are typically inorganic salts precipitating in an aqueous phase, such as calcium carbonate, calcium sulphate, barium sulphate and calcium oxalate.

According to the present invention it is, thus, possible to reduce the thickness of the multi-layer paper without impairing the opacity by using a filler that comprises fibrils over which calcium carbonate has been precipitated. GB Patent No. 628603 describes a multi-layer paper or board, the top layer of which contains modified fibre bulk. The bulk has been produced by impregnating the pulp with calcium chloride, after which the manipulated bulk is put in contact with carbonate compound, which causes the calcium carbonate to precipitate on the fibres - not on the fibrils. In the case corresponding to that described in the GB Patent, the bulk has considerably poor strength properties. It is stated in the publication, that it would not be possible to produce paper from this material. Moreover, the bulk has very poor retention.

More specifically, the fibre product according to the present invention is mainly characterised by what is stated in the characterising part of the claim 1.

The process according to the present invention, for its part, is characterised by what is stated in the characterising part of claim 8.

The present invention provides considerable advantages. Thus, a white lined liner can be prepared with a lighter top layer without compromising the strength of the surface. With the help of a new kind of a composite filling agent, the proportions of the white and brown layers can be changed much more easily. As the filler content can be increased and as the filler is extremely white, the amount of the white layer can be significantly decreased. By decreasing the white fibre layer, the commercial manufactures of liners can also decrease the total grammage of the liner. For example, it should be mentioned, that the grammage of the top layer according to the present invention can be at least about 5 % by weight, preferably at least 10 % by weight smaller than a top layer that has a corresponding opacity and formation and is prepared from the same fibre material and mineral pigment.

The filler has been found to improve the formation and stiffness of the top layer. The filler described in the FI Patent Specification No. 100729, referred hereinafter with its product name "SuperFill", retains well, which makes it possible to reduce the dosage of retention agents and still maintain a purer process. The better retention helps also to optimise/decrease the dosage of other paper making additives. Purity helps the operation of the machine and generally the operation efficiency of the machine improves, as the frequency of breaking down is smaller.

The present invention will be examined below in greater detail with the help of a detailed description and some examples.
Figure 1 present a side view of the principal structure of a two-layer fibre product and Figure 1b the corresponding four-layer fibre product,
Figure 2 shows the light scattering factor of a two-layer fibre product produced according to the present invention and two reference products as a function of the Mullen indices with two different filling factors,
Figure 3 shows corresponding results as a function of the bonding power (ScottBond),
Figure 4 shows corresponding results as a function of the tensile index, and
The figure 5 uses bar graphs to present the brightness of four two-layer fibre products, wherein two has top layers that contain filler according to the present invention, and two other contain reference filler.

### Filler and its preparation

As stated above, according to the present invention, composite filler comprising cellulose fibrils, on which light scattering pigments have been precipitated, is added as filler to the top layer of the multi-layer fibre product. Fibrils can originate from chemical pulp or mechanical pulp or mixtures thereof. By chemical pulp reference is herein made to a pulp, which has been treated with cooking chemicals to delignify cellulose fibres. According to a preferred embodiment the fibrils are obtained by refining pulps produced with the sulphate process or with some other alkaline cooking method. In addition to chemical pulps, fibrils can originate also from chemi-mechanical or mechanical pulps.

Typically, the average thickness of cellulose or lignocellulose fibrils is smaller than 5 µm, conventionally smaller than 1 µm. The fibrils are characterized by at least one of the following criteria:
a. they correspond to a fraction which passes a 100-mesh screen; and
b. their average thickness is 0.01 to less than 5 µm (preferably less than5 µm and in particular at maximum 1 µm) and their average length is 10 - 1500 µm.

The source material for the fibrils, i.e. the fines based on cellulose or other fibers, is fibrillated by beating it in a pulp refiner. The desired fraction may, when necessary, be separated by using a screen, but fines need not always be screened. Suitable fibril fractions include wire screen fractions P50 - P400. Preferably refiners with grooved blades are used.

The light-scattering material particles in the filler are inorganic or organic salts that can be formed from their source materials by precipitation in an aqueous medium. Such compounds include calcium carbonate, calcium oxalate, calcium sulphate, barium sulphate, and mixtures thereof. The material particles are deposited on the fibrils. The amount of an inorganic salt compound in proportion to the fibril amount is approx. 0.0001 - 95 % by weight, preferably approx. 0.1 - 90 % by weight, most suitably approx. 60 - 80 % by weight, calculated from the amount of filler, and approx. 0.1 - 80 % by weight, preferably approx. 0.5 - 50 % by weight, of the paper.

In the following, the present invention is examined with particular reference to a product according to FI Patent Specification No. 100729, but it is clear that the present invention can be adapted for other products mentioned hereinbefore by changing appropriately the source materials of the light scattering pigment.

The filler is produced by precipitating a mineral pigment on the surface of fine fibrils prepared from cellulose fibres and/or mechanical pulp fibres. For example, the precipitation of calcium carbonate can be carried out by feeding into an aqueous slush of fibrils an aqueous calcium hydroxide solution which possibly contains a solid calcium hydroxide, and a compound which contains carbonate ions and is at least partly dissolved in water (e.g. sodium carbonate or ammonium carbonate). It is also possible to introduce into the aqueous phase carbon dioxide gas that, in the presence of calcium hydroxide, produces calcium carbonate. There are formed string-of-pearls-like calcium carbonate crystal aggregates, which are held together by fibrils, i.e. fine strands, and in which the calcium carbonate particles are deposited onto the fine fibrils and attached to them. The fine fibrils together with calcium carbonate form string-of-pearls-like strands, and the calcium carbonate aggregates primarily resemble strings of pearls in a pile. In water (slush) the ratio of the effective volume of the aggregates to the pulp is very high compared with the corresponding ratio of conventional calcium carbonate used as filler. By "effective volume" is meant, in this case, the volume required by the pigment.

The diameter of the calcium carbonate particles in the aggregates is about 0.1 to 5 µm, typically about 0.2 to 3 µm. In particular, the fibrils correspond to wire screen fractions P50 (or P100) to P400.

1 to 90 % by weight (dry weight), typically about 5 to 50 % by weight, of this kind of filler is added to the top layer of a multi-layer product. Usually the filler described forms at least 5 % by weight, most suitably from 10 to 100 % by weight of the filler of the base web and respectively 10 to 50 % by weight of the fibre material of the base web. In principle it is also possible to produce a base web the fibre material of which consist totally of fibrils of the filler, so, in general, the present filler can form 1 to 100 % by weight of fibre material of the base web.

In the slush used in the production of the bottom web, part of the filler can consist of conventional fillers, such as calcium carbonate. However, preferably at least 80 %, especially preferably at least 90 % of the precipitated light scattering pigment particles are attached into the fibrils.

### Multi-layer structure

Figures 1a and 1b illustrate the structures of the multi-layer products containing two and four layers, respectively. Figure 1a illustrates a typical white lined liner board and Figure 1b illustrates so called test liner.

The grammage of the fibre product according to the present invention is preferably about 50 to 500 g/m², typically about 80 to 350 g/m². Usually its grammage is over 125 g/m², but products having a grammage below 100 g/m² qualify for small packages.

Preferably the liner according to the present invention comprises a two-layer product (see Figure 1a), that has a surface of a cover layer 1 and a back layer 2. The top layer covers the back layer so that the back layer cannot be seen through the top layer.

It is also possible to produce three-layer or four-layer products. In principle the number of layers in a layer product has no upper limit, there can be even up to 5, 6 or 7 layers. What is essential in the present invention, is that the top layer contains filler described more precisely hereinbefore, so that the top layer covers the layers under it, the layers that can be produced from raw materials of cheap costs.

Among multi-layer products, the test liner type four-layer products of Figure 1b, having a top layer 3, a layer 4 under the top layer, intermediate layer 5 and a back layer 6, are to be mentioned.

Different raw materials can be used for production of a fibre product according to the purpose of use. Both virgin fibres and recycled fibres can be used. The virgin fibre can originate from softwood or hardwood (wood chips) or it can originate from cuttings. Especially preferably virgin pulp is used in the top layer. This is most suitably produced by sulphate cooking (kraft pulp), because sulphate cooking gives a mass having especially good strength properties, as the name suggests. The recycled fibre can originate e.g. from used corrugated board packages (OCC) or mixed fibres. Recycled fibres are used especially for the production of test liners. The surface and back layer(s) can be produced from similar raw materials or from different source fibres. If virgin fibre, such as kraft pulp, is used for both, then the mass of the back layer can be cooked in high yield, after which a mild refining is performed on it. Mass that has been cooked to a lower kappa and also refined more than mass of the back layer, is used for the top layer. Typically the pulp of the back layer is cooked to a kappa value of 30 to 70 and the pulp of the top layer to lower kappa value of 25 (the kappa number of the unbleached pulp). Bleaching can be performed in a manner known per se, e.g. as ECF of TCF bleaching.

Retention agents can be added to the slush e.g. in about 0.5 to 3 % of the amount of the fibre material. However, it has been found in connection with the present invention that the filler described here gives such a good retention that no retention agents are needed for the layer the and amount of the retention agents can be significantly decreased. The liner is stuff or surface sized to improve the moisture resistance. If a low quality recycled fibre is used as raw material, it is preferable to use a surface-size press to produce a product that has sufficient strength. According to the machine the distribution of the base weight between the top and the back layer is about 20/80...40/60, typically about 30/70. Thus the grammage of the top layer is generally about 20 to 125 g/m² (see below). When operating according to the present invention, the grammage of the top layer can be decreased over 10 %, up to 20 % or more, without deteriorating the optical or mechanical properties of the cover.

The layer product is produced in a manner known per se. According to one preferred embodiment both or all layers are produced first from slush of their own and spread on the Fourdriner wire. After this, the layers are couched fastened into each other. With regard to the production process, a reference is made to a text by Ari Kiviranta "Board Grades", in a book series Paper Making Science and Technology, Book 18, Paper and Board Grades, Fapet Oy, Jyväskylä 2000, pages 68 and 69.

A planar fibre product according to the present invention can be used as a top layer of different corrugate board packages. The solution according to the present invention is especially preferably suitable for white lined top liner and coated white lined liner, both of which are used for demanding printing works. In these objects the fact that the surface of the liner according to the invention is extremely smooth and uniform, and has at the same time high opacity and brightness can be made use of. Generally the grammage of the top layer is about 20 to 125 g/m², most suitably about 50 to 80 g/m², especially preferably about 55 to 70 g/m², and bleached chemical cellulose pulp is used of the top layer. In order to obtain a very good formation in the preferred embodiment of the present invention, mainly hardwood is used in the top layer. Thus e.g. over 60 % by weight, typically over 80 % of fibre material of pulp is hardwood and the rest softwood. The fibre material of pulp can consist totally of hardwood.

Conventional coating mixtures can be used for coating of the coated white lined top layer product. Precipitated calcium carbonate, ground calcium carbonate, calcium sulphate, calcium oxalate, aluminium silicate, kaolin (hydrous aluminium silicate), aluminium hydroxide, magnesium silicate, talc (hydrous magnesium silicate), titanium dioxide and barium sulphate, and mixtures thereof can be used as pigments. Synthetic pigments can also be used. Of the pigments mentioned above, the main pigments are kaolin, calcium carbonate, precipitated calcium carbonate and gypsum, which in general constitute over 50 % of the dry solids in the coating mix. Calcined kaolin, titanium dioxide, satin white, aluminium hydroxide, sodium silicoaluminate and plastics pigments are additional pigments, and their amounts are in general less than 25 % of the dry solids in the mix. Special-quality kaolins and calcium carbonates, as well as barium sulphate and zinc oxide of the special pigments should be mentioned as examples.

Any known binders generally used in paper production can be used as binders in the coating composition. Besides the individual binders, it is also possible to use mixtures of binders. Examples of typical binders include synthetic latexes made up of polymers or copolymers of ethylenically unsaturated compounds, e.g. copolymers of the butadienestyrene type, and polyvinyl acetate having comonomers that contain carboxyl groups. Together with the materials mentioned above, it is possible to use , for example, water-soluble polymers, starch, CMC, hydroxyethyl cellulose and polyvinyl alcohol as binders. Furthermore, conventional additives and auxiliary agents, such as dispersants, agents affecting the viscosity and water retention of the mix, lubricants, hardeners used for improving water-resistance, optical auxiliary agents, anti-foaming agents, pH control agents, and preservatives can be used in the coating composition.

The coating mix can be applied to the material web in a manner known per se. The coating can be done before couching. Preferably it is done after forming the multi-layer structure. The method according to the present invention for coating paper and/or board can be carried out with a conventional coating apparatus, in other words by blade coating, or by film coating or JET application. Coating can be done on-line or off-line.

The amount of grammage of the coating layer varies from 5 to 30 g/m².

It has also been found in the context of the present invention, quite surprisingly, that the above-described filler does not only improve opacity of the top layer but the filled layer is also very easy to be coated. The amount of pigment or amounts of coatings required for the desired brightness can be decreased with the filler.

According to the present invention, the opacity is significantly improved with the filler.

The following non-restrictive examples illustrate the present invention. The measurement results indicated for the paper properties in the examples have been determined by the following standard methods:
Surface roughness: SCAN-P76:95
Porosity: SCAN-P60
Resistance of air permeability: SCAN-M8,P19

### Example 1

### Production of filler

### Refining of chemical pulp

Birch sulphate pulp was refined with a Valmet JC-01 refiner to produce pulp that is suitable for production of filler. The consistency of refining was about 4 % and the total energy consumption was 343 kWh/t and specific edge load was 0.5 J/m.

Properties of the product are presented in Table 1.

**Table 1. Fibre properties before and after refining**

| | Before refining | After refining |
|---|---|---|
| Fibre length (length), mm | 0.86 | 0.58 |
| Fibre length (weight), mm | 1.00 | 0.77 |
| SR° | 16 | 86 |

### Carbonating of pulp

Carbonating was performed in tap water according to the FI Patent Specification No. 100729. Water slurry that has dry matter content of 2.22 % was produced. The final product had CaCO₃ content of 69.7 % and a specific surface area of 10.6 m²/kg.

### Example 2

Fibre layers suitable for cover layer of two-layer white lined liner was produced from chemical pulp that contained 70 % by weight of birch pulp and 30 % by weight of pine pulp. Filler was added from the pulp in the slush in various amounts: 13 and 20 % by weight, respectively, of filler described in example 1 (SuperFill), 14 and 16 % by weight, respectively, precipitated calcium carbonate (PCC, Albacar LO, ref. 1) and 14 % by weight of mixture of chalk and calcined kaolin (ref. 2).

Figures 2 to 4 illustrate the light scattering ability of the obtained fibre layers as a function of mechanical strength properties. The figures show that the light scattering factor is at least 25 % and about 20 % greater with the SuperFill filler when compared with references 1 and 2 in constant strengths.

Consequence of this is that the grammage of the surface can be decreased by about 20 %, which decreases significantly production costs of liner.

Figure 5 shows a result in which the above presented results are substantiated. The result is from a liner test run made by pilot machine (FEX) of STFI in Stockholm, wherein the grammage of the surface was decreased from the normal level of 75 g/m² to a level of 65 g/m². A two-layer fibre structure was produced for the test. The ISO brightness of the product was determined.

Figure 5 shows that the top layer lightened 10 g/m² with Superfill, generates brightness which is 4 brightness units greater as compared with the reference 2, in which the grammage is 75 g/m². The result is extremely good and it suggests that the grammage of the surface can be decreased even lower than 10 g/m².

## Claims

1. A multi-layer fibrous product comprising of at least two overlapping fibre layers (1, 2; 3-6), of which the one (1; 3), which forms the top layer, contains fibres from a chemical cellulose pulp, and a filler, and is lighter than the layer under it (2; 4-6) and is opaque, **characterised in that**
- the top layer (1; 3) is produced from chemical cellulose pulp comprising hardwood pulp, softwood pulp or a mixture thereof;
- the filler of the top layer (1; 3) consists at least partially of cellulose or lignocellulose fibrils, on which light scattering material particles of inorganic or organic salts have been precipitated in an aqueous medium, wherein said fibrils are produced by refining and screening from plant fibres, the average thickness of the fibrils being less than 5 µm;
- the back layer comprises 1 to 5 layers (2; 4-6) that have been produced from virgin fibre or recycled fibre; and
- the distribution of the grammage between the top and back layers is 20/80 to 40/60.

2. A fibrous product according to claim 1, **characterised in that** the light scattering material particles has been precipitated over fibrils corresponding to a fraction that passes through a 50 mesh screen and/or having an average thickness of 0.01 to less than 5 µm and an average length of 10 to 1500 µm.

3. A fibrous product according to claim 1 or 2, **characterise**d in that the light scattering material particles are inorganic salts that can be formed from their source materials by precipitating in an aqueous medium.

4. A fibrous product according to claim 3, **characterised in that** the light scattering material particles are calcium carbonate, calcium oxalate, calcium sulphate, barium sulphate or mixtures thereof.

5. A fibrous product according to any of the preceding claims, **characterised in that** it comprises white lined top liner or coated white lined liner.

6. A fibrous product according to any of the preceding claims, **characterised in that** its grammage is preferably about 50 to 500 g/m², typically about 80 to 350 g/m², in which case the grammage of the top layer is about 20 to 125 g/m², preferably about 50 to 70 g/m².

7. A fibrous product according to any of the preceding claims, **characterised in that** the grammage of the top layer is at least about 5 % by weight, preferably at least 10 % by weight, less than the top layer that has been produced from the same fibre material and mineral pigments and that has corresponding opacity and formation.

8. A process for producing a multi-layer product according to any of claims 1 to 7, according to which process a filler-containing fibre layer, which forms the surface (1; 3) of the fibre product and covers the back layer, is fitted on top of a backing layer (2; 4-6) that consists of at least of one fibrous layer, **characterised in that**
- the top layer (1; 3) is formed from slush of fibre material, which is chemical cellulose pulp, to which a filler comprising cellulose or lignocellulose fibrils on which light scattering material particles have been precipitated, is added, wherein said fibrils are produced from plant fibres by refining and screening, said fibrils having an average thickness of less than 5 µm, the top layer (1; 3) being produced from chemical cellulose pulp comprising hardwood pulp, softwood pulp or a mixture thereof,
- the back layer comprising 1 to 5 layers (2; 4-6) that have been produced from virgin fibre or recycled fibre; and
- the distribution of the grammage between the top and back layers being 20/80 to 40/60.

9. A process according to claim 8, **characterised by** using a filler, in which the light scattering material particles have been precipitated on fibrils corresponding to a fraction that passes through a 50 mesh screen and/or having an average thickness of 0.1 to less than 5 µm and an average length of 10 to 1500 µm.

10. A process according to claim 8 or 9, **characterised by** using a filler in which at least 80 % of the precipitated light scattering pigment particles are attached to the fibrils.

11. A process according to any of the claims 8 to 10, **characterised in that** the top layer is coated in a paper machine with a pigment-containing coating mixture.

12. A method according to any of claims 8 to 11, **characterised in that** the top layer (1; 3) and the back layer(s) (2; 4-6) are formed separately on the Fourdriner wire and couched when still wet.

## Patentansprüche

1. Mehrschichtiges Faserprodukt, umfassend mindestens zwei sich überschneidende Faserschichten (1, 2; 3-6), von denen die eine (1; 3), welche die Deckschicht bildet, Fasern aus einem chemischen Cellulosezellstoff und einen Füllstoff enthält, und leichter als die darunter liegende Schicht (2; 4-6) und opak ist,
**dadurch gekennzeichnet, dass**
- die Deckschicht (1; 3) aus chemischem Cellulosezellstoff hergestellt ist, der Hartholzzellstoff, Weichholzzellstoff oder eine Mischung davon umfasst;
- der Füllstoff der Deckschicht (1; 3) mindestens teilweise aus Cellulose- oder Lignocellulosefibrillen besteht, auf denen lichtstreuende Materialteilchen aus anorganischen oder organischen Salzen in einem wässrigen Medium ausgefällt worden sind, wobei die Fibrillen durch Raffinieren und Sieben von Pflanzenfasern hergestellt werden, wobei die durchschnittliche Dicke der Fibrillen weniger als 5 µm beträgt;
- die Rückschicht 1 bis 5 Schichten (2; 4-6) umfasst, die aus Frischfaser oder Recyclingfaser hergestellt worden sind; und
- die Verteilung des Flächengewichts zwischen der Deck- und Rückschicht 20/80 bis 40/60 beträgt.

2. Faserprodukt nach Anspruch 1, **dadurch gekennzeichnet, dass** die lichtstreuenden Materialteilchen über Fibrillen ausgefällt worden sind, die einer Fraktion entsprechen, die ein Sieb mit einer Maschenweite von 50 mesh durchlaufen und/oder eine durchschnittliche Dicke von 0,01 bis kleiner als 5 µm und eine durchschnittliche Länge von 10 bis 1500 µm aufweisen.

3. Faserprodukt nach Anspruch 1 oder 2, **dadurch gekennzeichnet, dass** die lichtstreuenden Materialteilchen anorganische Salze sind, die aus ihren Ausgangsmaterialien gebildet werden können, indem sie in einem wässrigen Medium ausgefällt werden.

4. Faserprodukt nach Anspruch 3, **dadurch gekennzeichnet, dass** die lichtstreuenden Materialteilchen Calciumcarbonat, Calciumoxalat, Calciumsulfat, Bariumsulfat oder Mischungen davon sind.

5. Faserprodukt nach einem der vorstehenden Ansprüche, **dadurch gekennzeichnet, dass** es eine weiße ausgekleidete obere Auskleidung oder eine beschichtete weiße ausgekleidete Auskleidung umfasst.

6. Faserprodukt nach einem der vorstehenden Ansprüche, **dadurch gekennzeichnet, dass** sein Flächengewicht vorzugsweise etwa 50 bis 500 g/m², typischerweise etwa 80 bis 350 g/m² beträgt, wobei in diesem Fall das Flächengewicht der Deckschicht etwa 20 bis 125 g/m², vorzugsweise etwa 50 bis 70 g/m² beträgt.

7. Faserprodukt nach einem der vorstehenden Ansprüche, **dadurch gekennzeichnet, dass** das Flächengewicht der Deckschicht mindestens etwa 5 Gew.-%, vorzugsweise mindestens 10 Gew.-%, kleiner als die Deckschicht ist, die aus dem gleichen Fasermaterial und Mineralpigmenten hergestellt worden ist und die entsprechende Opazität und Formation aufweist.

8. Verfahren zur Herstellung eines mehrschichtigen Produkts nach einem der Ansprüche 1 bis 7, nach welchem Verfahren eine füllstoffhaltige Faserschicht, welche die Oberfläche (1; 3) des Faserprodukts bildet und die Rückschicht bedeckt, auf der Oberseite einer Trägerschicht (2; 4-6) aufgesetzt ist, die aus mindestens einer Faserschicht besteht, **dadurch gekennzeichnet, dass**
- die Deckschicht (1; 3) aus einem Schlamm aus Fasermaterial gebildet wird, bei dem es sich um einen chemischen Cellulosezellstoff handelt, dem ein Füllstoff, der Cellulose- oder Lignocellulosefibrillen enthält, auf denen lichtstreuende Materialteilchen ausgefällt worden sind, zugegeben wird, wobei die Fribrillen aus Pflanzenfasern durch Raffinieren und Sieben hergestellt werden, wobei die Fibrillen eine durchschnittliche Dicke von kleiner als 5 µm aufweisen, wobei die Deckschicht (1; 3) aus chemischem Cellulosezellstoff hergestellt ist, der Hartholzzellstoff, Weichholzzellstoff oder eine Mischung davon umfasst,
- die Rückschicht 1 bis 5 Schichten (2; 4-6) umfasst, die aus Frischfaser oder Recyclingfaser hergestellt worden sind; und
- die Verteilung des Flächengewichts zwischen der Deck- und Rückschicht 20/80 bis 40/60 beträgt.

9. Verfahren nach Anspruch 8, **gekennzeichnet durch** das Verwenden eines Füllstoffs, in dem die lichtstreuenden Materialteilchen auf Fibrillen ausgefällt worden sind, die einer Fraktion entsprechen, die ein Sieb mit einer Maschenweite von 50 mesh durchlaufen und/oder eine durchschnittliche Dicke von 0,1 bis kleiner als 5 µm und eine durchschnittliche Länge von 10 bis 1500 µm aufweisen.

10. Verfahren nach Anspruch 8 oder 9, **gekennzeichnet durch** das Verwenden eines Füllstoffs, in dem mindestens 80% der ausgefällten lichtstreuenden Pigmentteilchen an den Fibrillen angebracht sind.

11. Verfahren nach einem der Ansprüche 8 bis 10, **dadurch gekennzeichnet, dass** die Deckschicht in einer Papiermaschine mit einer pigmenthaltigen Beschichtungsmischung beschichtet wird.

12. Verfahren nach einem der Ansprüche 8 bis 11, **dadurch gekennzeichnet, dass** die Deckschicht (1; 3) und die Rückschicht(en) (2; 4-6) separat auf dem Fourdrinerkabel ausgebildet und im noch feuchten Zustand formuliert werden.

## Revendications

1. Produit fibreux multicouche comprenant au moins deux couches de fibres superposées (1, 2 ; 3-6), dont l'une (1 ; 3), qui forme la couche de dessus, contient des fibres provenant d'une pâte de cellulose chimique et une charge, et est plus légère que la couche sous-jacente (2 ; 4-6) et est opaque,
**caractérisé en ce que**
- la couche de dessus (1 ; 3) est fabriquée à partir de pâte de cellulose chimique comprenant de la pâte de bois dur, de la pâte de bois tendre ou un mélange de celles-ci ;
- la charge de la couche de dessus (1 ; 3) est constituée au moins en partie de fibrilles de cellulose ou de lignocellulose, sur lesquelles des particules de matériau diffusant la lumière de sels inorganiques ou organiques ont été précipitées dans un milieu aqueux, dans lequel lesdites fibrilles sont fabriquées par raffinage et criblage à partir de fibres végétales, l'épaisseur moyenne des fibrilles étant inférieure à 5 µm;
- la couche support comprend 1 à 5 couches (2 ; 4-6) qui ont été fabriquées à partir de fibres vierges ou de fibres recyclées ; et
- la répartition du grammage entre les couches de dessus et support est de 20/80 à 40/60.

2. Produit fibreux selon la revendication 1, **caractérisé en ce que** les particules de matériau diffusant la lumière ont été précipitées sur des fibrilles correspondant à une fraction qui traverse un tamis de 50 mesh et/ou ayant une épaisseur moyenne de 0,01 à moins de 5 µm et longueur moyenne de 10 à 1500 µm.

3. Produit fibreux selon la revendication 1 ou 2, **caractérisé en ce que** les particules de matériau diffusant la lumière sont des sels inorganiques qui peuvent être formés à partir de leurs matériaux sources par précipitation dans un milieu aqueux.

4. Produit fibreux selon la revendication 3, **caractérisé en ce que** les particules de matériau diffusant la lumière sont du carbonate de calcium, de l'oxalate de calcium, du sulfate de calcium, du sulfate de baryum ou des mélanges de ceux-ci.

5. Produit fibreux selon l'une quelconque des revendications précédentes, **caractérisé en ce qu'**il comprend un revêtement supérieur revêtu de blanc ou un revêtement revêtu de blanc enduit.

6. Produit fibreux selon l'une quelconque des revendications précédentes, **caractérisé en ce que** son grammage est de préférence d'environ 50 à 500 g/m², typiquement d'environ 80 à 350 g/m², auquel cas le grammage de la couche de dessus est d'environ 20 à 125 g/m², de préférence d'environ 50 à 70 g/m².

7. Produit fibreux selon l'une quelconque des revendications précédentes, **caractérisé en ce que** le grammage de la couche de dessus est d'au moins environ 5% en poids, de préférence d'au moins 10% en poids, inférieur à la couche de dessus qui a été fabriquée à partir des mêmes matériau fibreux et pigments minéraux et qui présente une opacité et une formation correspondantes.

8. Procédé de fabrication d'un produit multicouche selon l'une quelconque des revendications 1 à 7, selon lequel une couche de fibres contenant une charge, qui forme la surface (1 ; 3) du produit fibreux et recouvre la couche support, est placée au-dessus d'une couche de renfort (2 ; 4-6) constituée d'au moins une couche fibreuse, **caractérisé en ce que**
- la couche de dessus (1 ; 3) est formée à partir de boue de matériau fibreux, qui est une pâte de cellulose chimique, à laquelle une charge, comprenant des fibrilles de cellulose ou de lignocellulose sur lesquelles des particules de matériau diffusant la lumière ont été précipitées, est ajoutée, dans lequel lesdites fibrilles sont fabriquées à partir de fibres végétales par raffinage et criblage, lesdites fibrilles ayant une épaisseur moyenne inférieure à 5 µm, la couche de dessus (1 ; 3) étant fabriquée à partir de pâte de cellulose chimique comprenant de la pâte de bois dur, de la pâte de bois tendre ou un mélange de celles-ci,
- la couche support comprenant 1 à 5 couches (2 ; 4-6) qui ont été fabriquées à partir de fibres vierges ou de fibres recyclées ; et
- la répartition du grammage entre la couche de dessus et des couches support étant de 20/80 à 40/60.

9. Procédé selon la revendication 8, **caractérisé par** l'utilisation d'une charge dans laquelle les particules de matériau diffusant la lumière ont été précipitées sur des fibrilles correspondant à une fraction qui traverse un tamis de 50 mesh et/ou ayant une épaisseur moyenne de 0,1 à moins 5 µm et une longueur moyenne de 10 à 1500 µm.

10. Procédé selon la revendication 8 ou 9, **caractérisé en ce que** l'on utilise une charge dans laquelle au moins 80% des particules de pigment diffusant la lumière précipitées sont fixées aux fibrilles.

11. Procédé selon l'une quelconque des revendications 8 à 10, **caractérisé en ce que** la couche de dessus est revêtue dans une machine à papier avec un mélange de revêtement contenant un pigment.

12. Procédé selon l'une quelconque des revendications 8 à 11, **caractérisé en ce que** la couche de dessus (1 ; 3) et la ou les couches support (2 ; 4-6) sont formées séparément sur le fil Fourdrinier et couchées lorsqu'elles sont encore mouillées.
